

Jan. 9, 1923.

1,441,479

W. BENNETT.  
PROCESS FOR MAKING AN ALLOYING ALLOY.  
FILED SEPT. 8, 1922.



Inventor  
Wilson Bennett  
By  
Marking Clerk  
Attorneys

## UNITED STATES PATENT OFFICE.

WILSON BENNETT, OF WELLINGTON, NEW ZEALAND.

## PROCESS FOR MAKING AN ALLOYING ALLOY.

Application filed September 8, 1922. Serial No. 586,998.

*To all whom it may concern:*

Be it known that I, WILSON BENNETT, a citizen of New Zealand, residing at Wellington, New Zealand, have invented certain new 5 and useful Improvements in Processes for Making an Alloying Alloy, of which the following is a specification.

This invention relates to the process of making an alloying alloy referred to in my 10 application for patent 572,100 filed June 30, 1922.

In that application I pointed out the advantages of making my alloying alloy of chromium, etc., directly from the ores, thus 15 obviating the step of previously refining the ores of chromium in making my alloying alloy.

An object of the present invention is to produce this alloying alloy in a continuous 20 process and without removing the alloying alloy from the furnace in which it is produced.

With this and other objects in view which will appear as the description proceeds, the 25 invention consists of the novel features hereinafter described in detail, illustrated in the annexed drawing and more particularly pointed out in the appended claims.

Referring to the drawings wherein the 30 same letters represent corresponding parts in the different views:—

Figure 1 is a sectional view of a suitable furnace for use in carrying out my invention with the electric circuits and contacts 35 diagrammatically shown connected to the furnace;

Fig. 2 is a section of the furnace at right angles to Fig. 1; and,

Fig. 3 is a sectional view of a detail of the 40 water cooled bottom electrode.

A and B are carbon electrodes and C is a water cooled electrode in the bottom of the furnace, said bottom being preferably lined with a magnesite material O, the rest of the 45 body of the furnace being the ordinary material. The electrode C, I preferably make of metal of approximately the same composition as the alloy formed in this furnace.

D, E, F, G, H and J represent switches, 50 the special functions of which will be later referred to in detail. They may be closed or opened to make or break certain circuits leading from a transformer K to the electrodes A, B and C. The electrodes A and 55 B may be supported by an arm L which in turn is supported on a standard P attached

to the side of the furnace or supported on a base at the side of the furnace. This standard is screw-threaded at its upper end at Q and a screw extended from an upper part M 60 attached to the arm L so that when the screw is rotated by a handle R the electrodes A and B will be raised and lowered in the furnace for a purpose to be described hereafter.

65

N are diagrammatical representations of a water tube passing upwardly and then horizontally and downwardly through the bottom of the electrode C, and water passed through the tube N will serve the purpose 70 of keeping cool the electrode C during the operation of the furnace.

I have discovered that certain metals and metalloids when alloyed together exercise a very beneficial effect in minimizing the rusting or corrosive properties of iron, when these metals and metalloids are present in certain predetermined quantities, for example, I have found that chromium, nickel, 75 copper, molybdenum, vanadium and silicon, when added in certain percentages to iron, produce a ferrous alloy highly impervious to rust and corrosion, in addition to adding exceptional physical properties, such as the ability of withstanding the action of acids, 80 alkalis and gases to a marked degree.

I have also found that these alloys are suitable to both hot and cold working and can be readily manufactured into shapes to meet the requirements of ordinary commercial use.

In order that the iron alloys shall most advantageously possess the qualities herein described, it is necessary that the constituent metals be substantially free from carbon, 95 sulphur, manganese and phosphorus, which seriously interfere with the working properties of the iron alloy, a carbon content of one per cent being the maximum amount. It is even preferable to obtain an iron alloy 100 with a carbon content of less than one per cent. Indeed, the total of carbon, sulphur, manganese, and phosphorus content should not exceed 0.885 per cent when taken in the aggregate.

A suitable composition for my improved iron alloy is chromium 9 to 20 per cent; nickel 0.5 to 3 per cent; copper 0.20 to 2 per cent; molybdenum 0.5 to 2 per cent; vanadium 0.25 to 2 per cent; silicon 0.5 to 2.5 per cent with carbon, sulphur, manganese and phosphorus not to exceed 0.885 per cent

105

110

when taken in the aggregate, the balance by difference being iron.

A suitable base for making my iron alloy is refined iron produced by any suitable ingot iron or steel making process as free as practical from carbon, manganese, sulphur, and phosphorus. The chromium, nickel, copper, molybdenum, vanadium and silicon may be added in the metallic and metalloid form, or for economy's sake, I prefer to add them in the form of ores, or ferrous alloys of all these metals and metalloids, either singly or in combination. Nickel and copper may be added in the form of cupric-nickel metal such as Monel metal.

In carrying out my entire process I take as a base, decarbonized and refined iron such as is used for ingot iron or steel manufacture, which may be produced in the ordinary manner in an open hearth furnace, care being taken to eliminate carbon, manganese, sulphur and phosphorus to the lowest possible extent. To the molten iron I add an alloying alloy of chromium, nickel, copper, molybdenum, vanadium and silicon in such percentages to produce the quantity and quality of the completed iron alloy desired, using aluminium as a deoxidizing, degasifying and solidifying agent.

30 My method of preparing the alloying alloys is of prime importance and I prefer to use the furnace illustrated in the drawing in making this alloying alloy.

To produce the alloying alloy I first intimately mix crushed chromite ore with coke and pile this charge of material around the electrodes A and B. This charge is then covered with a slagging material of lime and fluorspar. The furnace is then set into operation as an arc furnace by closing the switches E and either G, H or J, depending upon the amount of current that I wish passed through the electrodes A—B, the switches D and F being left open. This will produce an arc from the lower extremities of the electrodes A and B. The charge is completely melted and the result is a fused mass of chromium, iron, carbon and metalloids. This product is known commercially as ferro chromium. In this stage of the process the molten bath of metal will be found to be covered with a thick viscous slag containing percentages of chromium and iron oxides. This slag is now entirely removed and the second or decarburizing stage proceeded with. Upon the surface of the molten metal a quantity of crushed lime mixed with chromite ore, mill scale and silicon is thrown in to form a second slag. The chromite ore and mill scale are introduced as oxygen containing substances, and I have discovered that a high silicon content in the metal minimizes the chromium oxide losses in the slag to a marked degree which otherwise are relatively high when silicon is

not employed during the decarburizing process.

The electrodes A and B are now depressed so as to barely clear the metal surface, allowing only a small gap between the molten metal and the electrodes to prevent the metal bath from being impregnated by carbon from the electrodes. The furnace is now operated as a resistance or incandescent furnace with the upper electrodes A and B connected in parallel to one pole and the water cooled metal electrode C situated in the base of the hearth, connected to the opposite pole. This may be accomplished by closing switches D F and either G H or J, depending on the amount of current desired, and opening switch E. The temperature is raised and the decarburizing process proceeded with until a test piece shows the required carbon content of the finished alloy- 85 ing alloy.

The additional alloys of nickel, copper, molybdenum and vanadium should be introduced at this stage. They may be added in the form of metals or ferro alloys of these 90 metals, previously prepared. The chromium and iron contents of the metal bath should be determined and chromite ore or ferro chromium should be introduced if the chromium content should be found to be too low, 95 or iron scrap should be fed into the bath should the chromium content be found in excess of the desired amount. The decarburizing process is proceeded with until the carbon content required is obtained. In 100 practice it will be found that the components of the alloying materials are easily oxidized, especially the silicon and chromium. These oxidized products form a chromiferous silicate slag. This slag can be employed to 105 great advantage as fluxing material for subsequent meltings and decarburization.

The slag is carefully removed, leaving the metal bath with a clean surface. A covering of crushed lime is then thrown on the metal bath and the temperature of the furnace is raised to a point which will reduce the lime very quickly to a fluid state. When the lime slack is melted, coke dust is carefully thrown on top of the slag around and between the 110 electrodes A, B, care being taken not to allow coke to come in contact with the molten metal. The upper electrodes A, B, are elevated and the furnace operated as an arc furnace at high temperature to form a calcium carbide covering of the lime and coke. Immediately the coke dust is thoroughly incorporated with the lime, the upper electrodes are lowered to slightly above the metal bath surface as before described by 115 turning the handle R and operating the screw to lower the electrodes, and the furnace is then operated as a resistance or incandescent furnace, setting up a flow of metal under the calcium carbide flux. This 120 125 130

- is the third stage of the process and will be found in practice to speedily eliminate sulphur, phosphorus, manganese and silicon to an extremely low degree. The completed 50 alloying alloy is then run into the ladle and the refined iron previously referred to as obtained from the open hearth furnace is poured directly into the mixture.
- It is very desirable in order to obtain satisfactory results that the completed iron 10 alloy be made with accuracy, and to insure that the resulting compound shall contain the proper proportions as specified. To attain this result a ladle with a suitable weighing attachment is advisable and the desired percentage, by weight, of the alloying alloy run into the ladle from the electric furnace. Into this molten mixture sufficient of the refined iron from the open hearth furnace is 15 poured to produce the quantity and quality of the completed iron alloy desired. Aluminium or silicon either, or both, being inserted into the ladle to act as a deoxidizing, degasifying and solidifying agent during 20 the mixing stage. The completed iron alloy is then run into ingots or suitable moulds to produce castings, transferred to soaking pits, rolled, pickled, annealed and manufactured into sheets and shapes in the usual 25 manner.
- It is evident that my invention permits of various modification, for example, the proportion of copper, nickel, molybdenum, vanadium or silicon may be changed considerably, and under certain conditions one or 30 more of these elements may be omitted, although I prefer to use them approximately in the percentages specified.
- I claim as my invention:—
1. The process of producing an alloying 35 alloy which consists in mixing chromium ores with ore reducing agents in an electric furnace, passing an electric arc through the mixture to reduce and refine the metals, removing the resulting slag, adding a decarbonizing mixture including a high content of silicon to the remaining metals and passing a current through the mass to reduce the 40 carbon to a low percentage and to eliminate excessive chromide oxide losses during the decarbonization, and removing the resulting slag.
2. A process of producing an alloying 45 alloy from ores, which consists in mixing chromite ores with a carbonaceous material, covering the same with a basic material, then passing an arc through the ores to melt and reduce the same, removing the slag then covering the metal with lime, chromium ore, mill scale and silicon, and subsequently passing a current through the same to reduce the carbon to a low percentage and to eliminate excessive chromide oxide losses during the decarbonization.
3. The process of making an alloying 50 alloy as set forth in claim 1 and adding to the metal some form of nickel, copper and silicon.
4. The process of making alloying alloy 55 as set forth in claim 1, and adding to the metal some form of nickel, copper, molybdenum, vanadium and silicon.
5. The process of making an alloying 60 alloy comprising mixing the ores of chromium with a carbonaceous material, covering the same with a slagging material and passing an electric arc therethrough, removing the slag thus formed, covering the top of the metal with lime, a chromium ore, mill scale and silicon, passing a current through the mixture to rid the alloy of its carbon content as described.
6. The process set forth in claim 5, together with the step of adding some form of nickel and copper to the resulting alloy.
7. The process set forth in claim 5 together with the step of adding nickel, copper, molybdenum and vanadium to the alloy formed.
- In testimony whereof I affix my signature 70 in presence of two witnesses.

WILSON BENNETT.

Witnesses:

CHAS. B. COMPTON,  
STEWART L. WHITMAN.